

# UNITED STATES PATENT OFFICE.

ERNEST FAHRIG, OF PHILADELPHIA, PENNSYLVANIA, ASSIGNOR OF ONE-HALF TO  
A. D. CLARK, OF PHILADELPHIA, PENNSYLVANIA.

## ARTIFICIAL SLATE.

1,362,563.

Specification of Letters Patent. Patented Dec. 14, 1920.

No Drawing.

Application filed December 10, 1919. Serial No. 343,961.

To all whom it may concern:

Be it known that I, ERNEST FAHRIG, a citizen of the United States, residing in Philadelphia, Pennsylvania, have invented 5  
Artificial Slate, of which the following is a specification.

One object of my invention is to provide a novel composition primarily intended to possess the qualities of and serve as a substitute for slate and which may be capable of being turned, polished and otherwise worked into any desired shapes, which shall be a good insulator, oil, acid and fire proof, hard, durable, structurally strong and water 15 resisting.

I further desire to provide a composition which while having the above noted qualities shall consist largely of slate, thus making it possible to utilize slate waste.

20 In the preferred form of my invention I prepare an intimate mixture of the following ingredients, in the specified proportions by weight, viz.,—slate 41%, sulfur 15%, quartzite, 11%, magnesite 10%, talc 9%, kaolin 8% and sericite 6%. Each of these 25 ingredients prior to mixture is first crushed to a half inch size and is then screened, after which it is operated on in a tube mill or other suitable pulverizing machine 30 whereby it is reduced to such a fineness that it will all pass through a one-hundred or higher mesh sieve. After being thus pulverized the materials specified are preferably stored separately in suitable bins where they 35 are maintained in a dry condition.

When it is desired to prepare a batch of the particular compound forming my invention, I charge a tube mill, for example, with the necessary weights of the above 40 noted ingredients in the proportions specified and operate such mill until said materials are so intimately mixed that an analysis of the product delivered shows that said in-

gredients are present in the proportions desired. When the mixing operation is complete, the finely pulverized mixture has added to it a suitable binder such as a 45 solution of one part aluminum chlorid and two parts magnesium chlorid having a specific gravity of 1.2 $\frac{1}{2}$  or higher, which is employed in such quantities as to render the product sufficiently plastic to permit it to be molded, pressed, cast or otherwise shaped to the form desired.

50 After being thus shaped the compound is allowed to dry or set until it has attained the desired hardness, when it may be turned, polished, sawed or otherwise worked into a desired form such as roofing or other tiles, blocks for use in walls or partitions, tool 55 handles, containers, etc.

Obviously other binders such as sodium silicate may be employed to obtain specific results without departing from my invention and various colors or pigments may be 60 added with the binder in order that the final product may possess the color desired.

I claim:

1. A composition of matter containing slate and sulfur in a powdered condition 70 as its principal ingredients together with a binder.

2. A composition of matter containing a predominance of slate, together with sulfur, quartzite, magnesite, kaolin, sericite, and 75 talc.

3. A composition of matter consisting of substantially 41% slate, 15% sulfur, 11% quartzite, 10% magnesite, 9% talc, 8% kaolin, 6% sericite, and a binder. 80

4. A composition of matter consisting mainly of slate and sulfur with other inert ingredients all in a powdered condition and a binder.

ERNEST FAHRIG.